

# UNITED STATES PATENT OFFICE.

JOHN WOOD LEADBEATER, OF LEEDS, ENGLAND.

## COMBUSTIBLE COMPOUND.

SPECIFICATION forming part of Letters Patent No. 622,374, dated April 4, 1899.

Application filed November 18, 1897. Serial No. 659,008. (No specimens.)

To all whom it may concern:

Be it known that I, JOHN WOOD LEADBEATER, engineer, a subject of the Queen of Great Britain and Ireland, residing at 55 Bannister Grove, Roundhay road, Leeds, in the county of York, England, have invented an Improved Combustible Compound, of which the following is a specification.

This invention has reference to a mode of bringing petroleum—that is to say, any known or available mineral oils—into a marketable form as a combustible other than in the ordinary liquid form; and it has for its object the manufacture of an insoluble compound having the essential quality of not melting and running during combustion, which compound may be in a condition hard enough to be handled and transported by rail, ship, or otherwise without danger and in a condition suitable for use as a combustible, or it may be in a condition somewhat approaching that of a fluid for mixing with other material along with which it is to act as a combustible.

I carry out my object as follows: I take a suitable quantity of petroleum, which may be crude or otherwise, (any mineral oil, residue, or refuse—for instance, "astatki"—will do,) and I add thereto a small proportion of animal or vegetable stearin—that is to say, a solid fat or solid fatty acid—resin, lime, and sawdust, (or other similar absorbent,) thoroughly mixing the whole with the application of as little heat as possible in order to minimize the evaporation of volatile matter. The said materials are hereinafter referred to shortly as "stearin," "resin," "lime," and "sawdust."

The proportions, which will vary according to circumstances, may be, for example, approximately as follows: To every one hundred and twenty-eight parts, by weight, of petroleum I add one part of animal or vegetable stearin, twelve parts of resin, eight parts of unslaked lime, and eight parts of sawdust, (preferably of a light and absorbent nature.)

The mode of mixing is preferably as follows: I first melt the stearin and the resin together in the same vessel, preferably in a steam-jacketed pan heated by low-pressure steam, using only the amount of heat necessary to melt the stearin and resin. (If desired to thin the mixture, a little of the petroleum may be added at this stage, taking care to use

as little heat as possible.) I mix the lime and the sawdust together, and I add them to and stir them in the petroleum, which, standing 55 in its independent vessel, is of course cold. The petroleum is thus absorbed by the sawdust. I then turn off the steam from the pan and add the mixture of petroleum, lime, and sawdust to the melted stearin and resin in the 60 pan, agitating the whole thoroughly to insure a proper admixture. After a short time a reaction will be noticed, accompanied by a rising of the mixture and a considerable increase of the temperature.

So far as I have been able to ascertain the action of the several ingredients is as follows: The sawdust not only serves as a combustible, but forms the main vehicle for absorbing the petroleum and mechanically holding it in suspension. The stearin and the resin melted together are ready to set up a saponifying action as soon as the lime is added, and these three assist in producing an insoluble result, (which, for instance, soda will not do.) As 75 the mixing takes place after the sawdust has been saturated with petroleum, the saponification resulting after the mixing mechanically closes up and seals the oil in the sawdust, and in this way the maximum amount of petroleum is dealt with. The water necessary for initiating the saponification is supplied by the "dry raw materials," so called in the ordinary sense, used for the manufacture of the material, and above all by the sawdust, (wood,) 80 which is preferably used in an entirely air-dried state, but still containing at least ten per cent. latent water and which parts with the moisture only on being moderately heated. Also the mineral oil contains in most cases 90 some dampness, so that the technically dry materials contain the quantity of moisture necessary for the initiation of the reaction. The addition of water is therefore unnecessary and even injurious, as it tends to leave 95 the finished product in a damp state and renders it soluble during combustion.

The resulting compound is insoluble, and when cold is a fairly hard waterproof substance; but if a harder or softer one be desired it may be made by using a different percentage of the ingredients. I therefore do not limit myself to the exact proportions of the various ingredients hereinbefore given.

This compound when prepared of the necessary stiffness and allowed to set hard may in the form of cakes or the like be handled, stored in heaps, and transported without danger in any suitable quantity or bulk, and it may after pulverization or division be used in that state as a fuel either in combination with other combustible matter or alone; or the ingredients may be proportioned so that the product when cold is in a state somewhat approaching that of a fluid, but which will set or practically set when mixed with other combustible materials. This admixture with other combustible materials may either take place immediately while the compound is still warm or at a remoter period when cold. The compound may be used as an enricher or as an assistant to an otherwise sluggish combustible when waste products of little calorific value are to be consumed, and in this latter way town's refuse, dried sewage sludge, and the like may be utilized in conjunction with the compound.

I make no general claim for treating petroleum with a view of solidifying or gelatinizing it, as my sole aim has been the introduction of a simple, inexpensive, and rapid mode of preparing a petroleum compound for use as

fuel that will not melt and run during combustion.

Having now particularly described and ascertained the nature of my said invention and in what manner the same is to be performed, I declare that what I claim is—

1. An insoluble combustible compound consisting of a mixture of petroleum, stearin, resin, lime and sawdust. 35

2. An insoluble combustible compound consisting of a mixture of petroleum, stearin, resin, lime and sawdust in approximately the following proportions by weight, to wit: one hundred and twenty-eight parts of petroleum, one part stearin, twelve parts of resin, eight parts of lime and eight parts of sawdust. 40

3. The process of preparing an insoluble combustible compound, said process consisting in melting stearin and resin together, adding thereto lime, sawdust and petroleum, and then agitating the mass. 45

In testimony whereof I have signed my name to this specification in the presence of two subscribing witnesses.

JOHN WOOD LEADBEATER.

Witnesses:

WILLIAM SNOWDON,

ARTHUR SAMUEL RICKARDS.